

1

3,512,928

**PURIFICATION OF MAGNESIUM CHLORIDE SALTS FOR ELECTROLYTIC MAGNESIUM PRODUCTION**

Leland R. Lyons, Boulder City, and Walter R. McCormick, Jr., Las Vegas, Nev., assignors to National Lead Company, New York, N.Y., a corporation of New Jersey  
No Drawing. Filed June 29, 1967, Ser. No. 649,824  
Int. Cl. C01f 5/26, 5/30; C22d 3/08  
U.S. Cl. 23—91 3 Claims

**ABSTRACT OF THE DISCLOSURE**

Method of purifying metal chloride salts with respect to soluble and reactive oxygen containing compounds, comprising fusing said salts in the presence of a carbonaceous dispersion of a member of the group consisting of activated carbon, colloidal carbon and combinations thereof in amount sufficient to react with oxygen values of said compounds which are evolved in gaseous form from said bath.

This invention pertains to improvements in the production of magnesium metal by electrolysis of magnesium chloride in fused salt baths containing the same. The invention pertains more particularly to the substantial elimination from such baths and/or from fused salts employed in such baths, of oxygen bearing compounds which attack the anodes and/or refractory lining of the electrolysis cell.

In the production of magnesium by electrolysis of  $MgCl_2$  in fused salt baths, extreme purity of the bath is of critical importance. In particular, oxygen bearing materials or compounds present in the bath which react at bath operating temperatures with the carbon anodes or refractory lining of the electrolysis cell, result in shortened cell life, losses of current, and contribute to surface tension problems which interfere with coalescence and proper recovery of the magnesium metal produced.

I have found that sulfates in particular, present in the bath, attack the carbon anode and refractory lining of the electrolysis cell with deleterious effects as above noted. I have discovered in accordance with this invention that these sulfates or other oxygen bearing materials which are soluble in the bath, may be eliminated from the bath or from fused salts introduced into the bath, by appropriate additions thereto of carbon in a highly dispersed or reactive form, such as activated carbon, or carbon bearing materials which produce activated carbon in the bath at the bath operating temperature, such as organic matter from marine organisms which produce activated carbon char at bath operating temperatures. Other bath additions which I have found suitable, are such substances as molasses, which upon destructive distillation in the bath produces carbon particles of colloidal particle size, uniformly dispersed throughout the bath.

I find that such highly activated or colloidally dispersed carbon reacts selectively with any sulfates or other soluble and reactive oxygen bearing compounds present in the fused salt bath, to eliminate oxygen in gaseous form, such as  $CO$ ,  $CO_2$ ,  $SO_2$ , etc., thus either completely to eliminate the oxygen content from the bath, or alternatively to eliminate the reactive portions thereof and reduce the compound in question to a stable and insoluble oxygen bearing compound, as for example to reduce  $MgSO_4$  present in the bath to the insoluble compound  $MgO$  with gaseous elimination of  $SO_2$ ,  $CO$  and/or  $CO_2$ . In consequence of this selective action, attack on the carbon anodes or refractory lining of the electrolysis cell is substantially eliminated, since the highly activated form in

2

which such carbon is introduced into the bath reacts much more rapidly with oxygen bearing compounds present in the bath than do the carbon anodes and cell lining. I find in this connection that ordinary carbon such as anode carbon, even when finely ground, does not produce this selective action.

The preferred treatment of the salts employed in the bath for eliminating or rendering innocuous, oxygen bearing compounds present in the salts, is to pretreat them by fusion in the presence of the aforesaid activated or colloidal carbon dispersion or in admixture with an organic material productive thereof in the fused salt.

The activated or colloidal carbon dispersion should be present in the fused salt in at least the amount required to react with the oxygen values which are evolved as  $CO$  and/or  $CO_2$  and as  $SO_2$ .

The invention finds particular application to elimination of residual sulfate values from aqueous salt solutions containing magnesium chloride and sulfate values, which have been processed substantially to eliminate the sulfate values for recovery of the magnesium values as  $MgCl_2$ . Examples of this are naturally occurring brines, such as found in salt lakes, inland seas, salt wells, etc., which in general contain principally sodium, potassium and magnesium chlorides and/or sulfates. As described in a pending application of L. W. Ferris, Ser. No. 400,994, filed Oct. 2, 1964, a process for recovering magnesium or  $MgCl_2$  from such brine, consists in subjecting the brine to successive concentrations, first to eliminate principally the sodium values as  $NaCl$ , and thence principally the potassium values as potassium-magnesium double salts, leaving  $MgCl_2$  and  $MgSO_4$  in solution in the mother liquor, which is substantially desulfated by treatment with calcium chloride, with precipitation of  $CaSO_4$  which is removed by filtration. Upon further concentration of the resultant mother liquor, the residual potassium values precipitate as the double salt, carnallite, along with residual  $NaCl$ , to leave an essentially  $MgCl_2$  mother liquid, which is further concentrated and ultimately reduced to powder form by spray drying. The essentially  $MgCl_2$  powder thus produced nevertheless contains sufficient of the sulfate radical as upon fused salt electrolysis thereof to attack the electrolysis cell carbon anodes and refractory lining, unless either pretreated in fused state with sufficient activated carbon present or produced therein upon fusion, or added as such or in an organic material productive thereof, to remove the  $SO_4$  values, or unless sufficient such activated carbon is present, produced or introduced into the electrolysis cell along with the powdered  $MgCl_2$  to accomplish this result.

The following examples are illustrative of the invention.

**EXAMPLE I**

Samples of naturally occurring brines containing  $Na$ ,  $K$ ,  $Mg$ ,  $Cl$  and  $SO_4$  ions and organic residues of extinct marine life were processed in the manner above described to produce spray dried essentially  $MgCl_2 \cdot 1.5H_2O$  powders, part of which was melted as such, and part of which was further dehydrated in hot  $HCl$  gases and then melted. Analyses of the  $SO_4$  and  $C$  contents of each before and after melting produced the following data.

|                 | Percent $SO_4$ | Percent C |
|-----------------|----------------|-----------|
| Dried:          |                |           |
| Powder          | 0.12           | 0.33      |
| Melted          | <0.05          | 0.18      |
| HCl dehydrated: |                |           |
| Powder          | 0.10-0.13      | 0.35-0.37 |
| Melted          | <0.05          | 0.21-0.24 |

The data show that the dispersed carbon produced by melting the dried and the dried and dehydrated  $MgCl_2$

powders reduce the  $\text{SO}_4$  content to less than 0.05% in each instance, from initial values of about 0.1-0.13%.

#### EXAMPLE II

The effect of adding carbon in the form of molasses to the concentrated  $\text{MgCl}_2$  solution obtained by processing a naturally occurring brine in the manner above set forth, is shown by this example, wherein for each 100 grams of  $\text{MgCl}_2$  in solution, there was added in one test, 2 gms of epsom salts,  $\text{MgSO}_4 \cdot 7\text{H}_2\text{O}$ , and 0.5 gm. molasses of specific gravity 1.38, and in another test was added 1 gm. of epsom salts and 0.07 gm. of said molasses. The two test solutions were then spray dried, HCl dehydrated, and melted with results as to  $\text{SO}_4$  and carbon contents at various stages as follows:

| G. $\text{MgSO}_4 \cdot 7\text{H}_2\text{O}/100$<br>g. $\text{MgCl}_2$ | G. molasses/<br>100 g. $\text{MgCl}_2$ | Percent $\text{HCl}$ dehydrated as         |                          |              |                          |
|------------------------------------------------------------------------|----------------------------------------|--------------------------------------------|--------------------------|--------------|--------------------------|
|                                                                        |                                        | Percent $\text{SO}_4$ as<br>spray<br>dried | Percent<br>$\text{SO}_4$ | Percent<br>C | Percent<br>$\text{SO}_4$ |
| 2                                                                      | 0.5                                    | 0.85                                       | 0.99                     | 0.14         | 0.49                     |
| 1                                                                      | 0.07                                   | 0.49                                       | 0.50                     | 0.06         | 0.07                     |

These data show that the retained, highly dispersed carbon from the molasses decomposition reduced the sulfate contents by amounts of 50% and 86%, respectively.

What is claimed is:

1. The method of purifying magnesium chloride contaminated by impurities in the form of soluble and reactive oxygen-containing compounds which comprises, fusing said impure magnesium chloride in the presence of a carbonaceous dispersion of a member of the group consisting of activated carbon, colloidal carbon and combinations thereof, in an amount and for a time sufficient to

react with said compounds and form oxygen-containing gaseous compounds evolved from said bath as such.

2. The method according to claim 1, wherein said impurities includes residual sulfates and the evolved gases are carbon-oxygen and sulphur-oxygen compounds.

3. The method according to claim 1, wherein there is added to or present in said impure magnesium chloride, a carbon-containing organic material which produces a dispersed carbon residue on fusion thereof, which carbon residue reacts with said oxygen-containing compounds to form oxygen-containing gaseous compounds.

#### References Cited

##### UNITED STATES PATENTS

|    |           |         |                            |          |
|----|-----------|---------|----------------------------|----------|
| 15 | 1,331,688 | 2/1920  | Bailey et al. -----        | 23-91 XR |
|    | 1,798,091 | 3/1931  | Lichtenberger et al. ----- | 23-90 XR |
|    | 1,923,594 | 8/1933  | Suchy et al. -----         | 23-87 XR |
|    | 1,933,499 | 10/1933 | Moschel -----              | 23-91    |
| 20 | 3,098,722 | 7/1963  | Carlson et al. -----       | 23-87 XR |
|    | 3,148,950 | 9/1964  | Mugg -----                 | 23-224   |
|    | 3,218,122 | 11/1965 | Nelson et al. -----        | 23-87    |
|    | 3,305,302 | 2/1967  | Heuer -----                | 23-67    |

##### FOREIGN PATENTS

|    |         |        |                |
|----|---------|--------|----------------|
| 25 | 293,410 | 7/1928 | Great Britain. |
|----|---------|--------|----------------|

##### OTHER REFERENCES

Ser. No. 292,742, Beck et al. (A.P.C.), published July 1943.

EDWARD STERN, Primary Examiner

U.S. Cl. X.R.

23-87; 204-70